

## [54] LUBRICATING COMPOSITIONS INHIBITED FROM OXIDATION

[75] Inventors: **Enzo Rossi; Silvano Fattori**, both of San Donato Milanese, Italy[73] Assignee: **Snam Progetti**, San Donato, Milanese, Italy[22] Filed: **Sept. 15, 1972**[21] Appl. No.: **289,227**

## [30] Foreign Application Priority Data

Sept. 16, 1971. Italy..... 28711/71

[52] U.S. Cl..... 252/48.2, 252/45, 252/406,  
250/329 HS

[51] Int. Cl..... C10m 1/38

[58] Field of Search..... 252/45, 48.2, 406;  
260/329 HS, 329 F

## [56] References Cited

## UNITED STATES PATENTS

2,521,514 9/1950 Hartough et al..... 252/45 X  
2,704,275 3/1955 Brooks..... 252/45

Primary Examiner—W. Cannon

[57]

## ABSTRACT

A lubricating composition of mineral oil or synthetic oil is inhibited from oxidation by dissolving therein, at temperatures not higher than 80° C., from 0.001 to 10 per cent by weight of a derivative of thio-thiophthene which is represented by the general formula:



wherein R, R<sub>1</sub>, R<sub>2</sub> and R<sub>3</sub>, which may be the same or different, are members of the group consisting of hydrogen, alkyl, cycloalkyl, aryl, alkylaryl, arylalkyl, alkoxyaryl, alkoxyalkyl, and aroxyalkyl, or R<sub>2</sub> and R<sub>3</sub> are combined and together represent an alkylene radical of the -CH<sub>2</sub>- type joined directly or by an equal CH<sub>2</sub>-CH<sub>3</sub> group to the other alkylene radical.

6 Claims, No Drawings

# LUBRICATING COMPOSITIONS INHIBITED FROM OXIDATION

The invention relates to the inhibition of the oxidation of lubricating compositions, achieved through the use of particular additives which have shown extremely valuable advantages with respect to the ones normally used in the art.

It is well known that the high temperatures developed in the modern engines favour the oxidation of lubricants with formation of acid products which cause the corrosion of the metal surfaces with which they come to contact.

Furthermore, said oxidation products deposit either as pitch products or varnish, or as lacquers on said metal surfaces thus causing a decrease of the efficiency of the engine itself. For the purpose of avoiding, as much as possible these undesirable effects from the lubricants the so-called antioxidant additives are added, such as the sterically hindered phenols, aromatic amines, alkylphenols sulphides, dialkylphosphates of Ca, Ba, and Al and other numerous ones.

But the inconveniences due to oxidation were not actually removed in a satisfactory way.

Therefore it is an object of this invention to supply additives which are inhibitors of oxidation for a wide range of products, such as lubricating compositions containing mineral oils, obtained from the most different raw materials refined through acids or solvents or coming from hydrocracking, said additives being also suitable to inhibit from oxidation lubricating compositions containing synthetic bases, such as synthetic hydrocarbons, synthetic esters, silicones, hydrogenated polyolefins, polyalkylene oxides, alkylbenzenes, esters of phosphoric acid and others.

Now we have found that the above mentioned effects, and others which will become apparent in the course of the present specification, are attained through the utilization of thio-thiophthene derivatives, which are adapted to give lubricating compositions on oxidation resistance which is absolutely better than the one obtained with other known oxidation inhibitors.

The thio-thiophthene derivatives may be represented by the following general formula



wherein R, R<sub>1</sub> may be equal or different and represent a hydrogen atom or an alkyl, cycloalkyl, aryl, alkyl-aryl, aryl alkyl, alkoxyaryl, alkoxyalkyl or aroxyalkyl group, R<sub>2</sub> and R<sub>3</sub> may be equal or different and represent a hydrogen atom or an alkyl, cycloalkyl, aryl, alkyl-aryl, arylalkyl, alkoxy-aryl, alkoxyalkyl or aroxyalkyl group, or R<sub>2</sub> and R<sub>3</sub> are combined and together represent an alkylene radical of the -CH<sub>2</sub>- type joined directly or by an equal CH<sub>2</sub>-CH<sub>3</sub> group to the other alkylene radical.

Said antioxidant additives dissolve in the lubricating fluid by heating to a temperature not higher than 70°-80° C.

The amount of the derivatives of the thio-thiophthene which are used depends on various factors

such as the nature of the base and the presence of other additives.

The use of said additives is particularly advantageous since they are efficacious also at very low concentrations, of about 0.01 percent or less. Generally the thio-thiophthene are used in concentrations which range from the 0.001 percent to 10 percent by weight and preferably from the 0.01 to the 5 percent b.w.

The lubricants containing the antioxidants of the invention may also contain various other types of additives normally used, like detergents, dispersants, corrosion inhibitors and antirust, viscosity index improvers, sludge inhibitors, pour point depressants and also other antioxidants in the case it were desirable to improve the characteristics of the oxidation inhibition of compositions already containing antioxidant agents.

The preparation of the thio-thiophthene derivatives of the present invention is generally well known to the people skilled in the art. For instance the methods described by F. Arndt et al. (Chem. Ber. 1925, 58, 1633) and by M. Stawaux and N. Lozach (Bull. Soc. Chim. France, 1967, 2082) may be used.

The method of preparation consists in causing the triketones, dissolved generally in aromatic solvents, to react with P<sub>2</sub>S<sub>5</sub>.

The reaction mass is treated with aqueous NaOH and the desired product crystallizes out of the organic phase.

The inventive antioxidants may also be named as derivatives of thio-thiophthene, and they may also be named as trithio-1,5,6 S<sup>IV</sup> pentalenes.

To provide a better understanding of the invention and to demonstrate the advantages of it, the following illustrative examples are reported.

## EXAMPLE 1

To a flask with three necks provided with a stirrer and cooler, 10 g of di 1-methyl-5-p.methoxyphenyl-1,3,5-triketone dissolved in 1,000 ml of benzene and 20 g of P<sub>2</sub>S<sub>5</sub> were fed.

Boiling was maintained during about 2 hours.

After cooling a concentrated solution of NaOH was added and it was stirred for about 15'.

At the end the benzene phase was separated.

The residue was subjected to two further extractions with benzene. The benzene extracts were gathered, washed with H<sub>2</sub>O and concentrated by evaporating the benzene.

A red brown residue was obtained.

By recrystallizing from ethyl acetate crystals were obtained having a melting point of 219°-220° C (observed 221° C). The sulfur content calculated for the C<sub>13</sub>H<sub>12</sub>OS<sub>3</sub> product was 34.30 percent; the ones found through analysis was 33.9 percent.

## EXAMPLE 2

With the purpose of evaluating the antioxidant properties of the thio-thiophthene derivatives in lubricating compositions, some tests of oxygen absorption were carried out. Said test was effected in an apparatus of the type described by G. Miliotis and co-operators (Bull. Soc. Chim. France, 1969; 847) and consisted in determining the induction period of the oxidation of a product maintained under a strong stirring in a reactor provided with a thermostat. The reactor filled with oxygen, was connected with a graduated buret for gases, which was also filled with oxygen.

A differential gauge marked the oxygen absorption. The tests were carried out at  $160 \pm 2^\circ\text{C}$  on 10 ml. oil samples, by using as catalyst copper powder in an amount of 50 mg.

The inventive products were dissolved in paraffinic mineral oil having a 30 SAE viscosity grade.

The results were reported in table 1.

TABLE 1

| Number of the test | Additive                                         | Concentration moles/liter | Induction period/minutes |
|--------------------|--------------------------------------------------|---------------------------|--------------------------|
| 1                  | none                                             | —                         | 14                       |
| 2                  | 2,6-di-t.butyl-4-methyl phenol                   | $10^{-2}$                 | 270                      |
| 3                  | 2.methyl-5-p.methoxyphenyl-thio-thiophthene      | $10^{-2}$                 | 638                      |
| 4                  | 2,5-di-p.methoxyphenyl-3-phenyl-thio-thiophthene | $10^{-2}$                 | 662                      |

## EXAMPLE 3

Through the apparatus and the method described in example 2 the additives of the invention dissolved in trimethyl adipate of octyl gave the results reported in table 2.

TABLE 2

| Number of the test | Additive                                             | Concentration moles/liter | Induction period, minutes |
|--------------------|------------------------------------------------------|---------------------------|---------------------------|
| 1                  | none                                                 | —                         | 4                         |
| 2                  | phenyl- $\alpha$ -naphthylamine                      | $3,5 \cdot 10^{-3}$       | 124                       |
| 3                  | 2-methyl-5-p.methoxyphenyl-thio-thiophthene          | $3,5 \cdot 10^{-3}$       | 148                       |
| 4                  | 2,5-di-p.methoxyphenyl-3-phenyl thio-thiophthene     | $3,5 \cdot 10^{-3}$       | 256                       |
| 5                  | 2,5-diphenyl-thio-thiophthene                        | $3,5 \cdot 10^{-3}$       | 220                       |
| 6                  | 2,5-di-p.methoxyphenyl-3,4-diphenyl-thio-thiophthene | $3,5 \cdot 10^{-3}$       | 197                       |
| 7                  | 2,5-di-phenyl-3,4-trimethylene-thio-thiophthene      | $3,5 \cdot 10^{-3}$       | 345                       |

The derivatives of thio-thiophthene may be advantageously used in oils for engines and for gears, in various hydraulic fluids and generally transmission fluids, in industrial and marine oils.

From tables 1 and 2 it is possible to notice that the compounds of the invention are remarkably better than well known commercial antioxidants such as 2,6-di-t.butyl-4-methyl-phenol and phenyl- $\alpha$ -naphthylamine.

Said derivatives of thio-thiophthene as already reported, particularly prevent the oxidation of various types of lubricating bases at high temperatures and achieve the purposes of the invention both as above mentioned from the point of view of a better activity as antioxidants with respect to the conventional antioxidants, and from the point of view of their flexibility in use as antioxidantizing agents in the already mentioned range of lubricating products.

We claim:

1. A lubricating composition, inhibited from oxidation, prepared by dissolving in an oil selected from the

group consisting of mineral and synthetic lubricating oils, at temperatures not higher than  $80^\circ\text{C}$  and in a quantity ranging from 0.001 to 10 per cent by weight, a derivative of thio-thiophthene represented by the general formula:



wherein R, R<sub>1</sub>, R<sub>2</sub> and R<sub>3</sub>, which may be the same or different, are members of the group consisting of hydrogen, alkyl, cycloalkyl, aryl, alkylaryl, arylalkyl, alkoxyaryl, alkoxyalkyl and aroxyalkyl, or R<sub>2</sub> and R<sub>3</sub> represent a CH<sub>2</sub>, CH<sub>2</sub>-CH<sub>2</sub> or CH<sub>2</sub>-CH<sub>2</sub>-CH<sub>2</sub> alkylene radical connecting the number 3 and 4 carbon atoms of the thio-thiophthene molecule.

2. Lubricating composition according to claim 1 characterized in that the derivative of the thio-thiophthene is 2-methyl-5-methoxyphenyl thio-thiophthene and is present in an amount in the range of 0.01 to 5 per cent by weight.

3. Lubricating composition according to claim 1 characterized in that the derivative of the thio-thiophthene is 2,5-di-p.methoxyphenyl-3-phenyl thio-thiophthene and is present in an amount in the range of 0.01 to 5 per cent by weight.

4. Lubricating composition according to claim 1 characterized in that the derivative of the thio-thiophthene is 2,5-diphenyl-thio-thiophthene and is present in an amount in the range of 0.01 to 5 per cent by weight.

5. Lubricating composition according to claim 1 characterized in that the derivative of the thio-thiophthene is 2,5-di-p.methoxyphenyl-3,4-diphenyl thio-thiophthene and is present in an amount in the range of 0.01 to 5 per cent by weight.

6. Lubricating composition according to claim 1 characterized in that the derivative of the thio-thiophthene is 2,5-di-phenyl-3,4-trimethylene-thio-thiophthene and is present in an amount in the range of 0.01 to 5 per cent by weight.

\* \* \* \* \*